

June 11, 1929.

F. K. L. SCHOUTEN  
PROCESS OF PRODUCING WOOD PULP

1,717,266

Filed March 2, 1927



Inventor:

Frans Karel Louis Schouten

by *W. V. Varek*  
his Attorney

Witnesses:

*W. G. Frenzen*

*H. Vlaardenburg*

## UNITED STATES PATENT OFFICE.

FRANS KAREL LOUIS SCHOUTEN, OF ZAANDAM, NETHERLANDS.

## PROCESS OF PRODUCING WOOD PULP.

Application filed March 2, 1927, Serial No. 172,045, and in Germany March 5, 1926.

The invention relates to the manufacture of wood pulp from logs or from wood waste, its object being to produce, by a mechanical process, pulp approximating in quality to hot ground.

According to my process the comminuted raw material, with its natural content of moisture, or moistened to restore the normal moisture content, is first subjected to so-called dry refining, and is then subjected to further refining (wet refining) in the presence of an appropriate proportion of added water. This process has the advantage of producing from logs or wood waste a pulp, which may be used in commerce in rolls, packets or as scrapings or the like, or may be subjected to further treatment, the pulp having in general the characteristic qualities of hot ground.

In carrying the invention into effect the raw material is disintegrated or opened up as thoroughly as may be, that is to say the bunches or bundles of fibre are sub-divided, the operation being continued till as far as convenient or practicable even the smallest bundles are divided into separate fibres. This may be done in three stages, to wit:—

*First stage.*—The raw material, holding its natural moisture content, is cut up or otherwise comminuted.

*Second stage.*—The comminuted material, still holding its natural moisture content, is subjected to dry refining.

*Third stage.*—In order finally to separate the fibres the material is subjected to wet refining, in the form of a thick pulp.

Logs, boards, wood shaving and so on may all be used as raw materials.

Such material may for the purposes of the process first be cut up into small slabs or wafers, which are then divided longitudinally of the fibres, the broken fibres and sawdust being separated, which may be done by any method usually adopted for that purpose, for example in a screen. Thereupon the fine woodflour, sawdust, sand and other impurities may be removed by sifting. Thereupon follows the already mentioned first refining process, namely a dry process, in which the wood holds only its natural moisture content. This effects disintegration into bundles of fibre, and is followed by the third stage of the process, namely wet refining.

If in the first stage of the process, up to the time when the material leaves the sifting apparatus, the moisture content has been unduly reduced, a certain proportion of mois-

ture may be introduced to restore the normal content, so that the mechanical treatment in the so-called dry refining process does not unduly tear the fibres.

The dry refining preceding the wet refining has the effect of dividing up the wood into bundles of fibres of fairly uniform size.

It is desirable for the purposes of the invention artificially to increase the heat produced by friction in the course of the dry refining process. For this purpose we may, for example, subject the beaters or coacting members of the refining apparatus to the action of springs or weights whereby their surfaces are pressed towards each other. The heat due to the resulting increased friction generates vapour in the wood, which opens up the cells. When the wood cells, thus loosened, are placed in the apparatus for wet refining, which imparts to the material the general characteristics of hot ground, the treatment produces a pulp capable of being made into paper with very closely felted fibre layers.

The treatment in the wet refiner disintegrates practically all the wood, even the smallest portions introduced into that apparatus, so that even these small bundles of fibres are opened up and converted into a loose fibrous state, as in hot ground. For this purpose the material on its way from the dry refiner to the wet refiner must be made into a pulp of such stiffness that its temperature is increased by friction in the wet refiner. This pulp may be produced in a vat, which is interposed between the dry and wet refiners, and from which the pulp is conveyed to the wet refiner by means of a suitable conveyor.

The thick pulp leaving the wet refiner may receive an addition of water, and then pass on to a sorting apparatus, wherein such bundles of fibres as have not been fully disintegrated or shredded are separated, in order to pass back to the vat and be mixed with the fresh material coming from the dry refiner. This prevents or reduces the occurrence of waste in the final stage of the process. The amount of water added to the material coming from the dry refiner is, of course, regulated with due regard to the water brought with the pulp which is returned to the vat after passing through the wet refiner and sorter. The water flowing from the sorting apparatus may, in fact, be used for regulating the consistency of the pulp which is supplied to the wet refiner.

An example of apparatus suitable for carrying the invention into effect is shown diagrammatically in the annexed drawing.

In the drawing 1 represents a machine for 5 comminuting the wood. This machine divides up the wood into small slabs in the manner customary in the wood pulp industry. The slabs of wood, and such other pieces as 10 pass out of the machine 1, pass into machines 2, which may, for example, be centrifugal machines or disintegrators, whereby the slabs are further divided. From the machines 2, the material passes to a sifting machine 3, wherein broken fibres and like waste material, 15 sand and other impurities are separated. This treatment completes the first stage.

For the second stage of the process the material passes into the dry refiner 6, where 20 the pieces of wood are divided up into coarse bundles of fibres, by being split longitudinally, heat being artificially generated by friction during this treatment.

If the material coming from the sifter is 25 too dry for this treatment it is first conveyed from the sifter to a chamber 5, wherein it is treated with water from a container 4, to restore the natural moisture content of the wood, whereupon it passes into the dry refiner 6, in which the second stage of the process is completed.

For the third stage the small bundles or 30 bunches of fibre produced in the dry refiner 6 are passed to vat 7, in order to convert into a pulp of the consistency suitable for wet refining. A pump 8 or equivalent apparatus 35 delivers this pulp to the wet refiner 9, in which the treatment, in so far as is practicable, is accompanied by artificial generation of heat by friction.

40 The pulp from the wet refiner, with addition of an appropriate quantity of water, passes to the sorting or straining apparatus 10, where any coarse material left in the pulp

is separated. The strained pulp passes on to the drier 11, and the water containing the 45 coarse matter flows back to the vat 7, and is mixed with the wood bundles, coming from the dry refiner.

The drier may, for example, be a single cylinder rotary strainer as used in cardboard 50 manufacture. The drier removes the appropriate proportion of water from the pulp, which is deposited in the form of sheets. The pulp may be bleached, for example, by the sodium disulphide process, if required, 55 and the material may if desired be converted in known manner into roll material or scrap ing material in these machines.

Presses, centrifugal apparatus or the like 60 may be used for further separation of water from the pulp, and putting it into packet form. A press for this purpose is shown at 12. From such a press the material can be taken in a form ready for the market, with a moisture content of only 50 to 55%. 65

Alternatively the pulp coming from the sorter or strainer can be thickened to the consistency suitable for treatment in a beater, and used for paper making, the treatment in the drier 11 and press 12 being dispensed 70 with.

What I claim is:

The process of mechanically producing 75 wood pulp comprising mechanically comminuting the raw material, dry refining it with sufficient friction to vaporize its normal water content, and wet refining it in mixture with added water controlled as to quantity so as to permit the frictional heat incident to the refining to elevate the temperature of the 80 mixture to such a point as to give to the pulp the character of hot-ground.

In testimony whereof I have affixed my signature.

FRANS KAREL LOUIS SCHOUTEN.